

1

3,375,061

## PYROHYDROLYTIC ATTACK OF RARE EARTH FLUOCARBONATE ORES

Robert M. Healy, Warrenton, Ill., and Lamar T. Royer, Oak Ridge, Tenn., assignors to American Potash & Chemical Corporation, Los Angeles, Calif., a corporation of Delaware

No Drawing. Filed Mar. 12, 1964, Ser. No. 351,511  
10 Claims. (Cl. 23—15)

### ABSTRACT OF THE DISCLOSURE

A process for recovering substantially all of the rare earth values from rare earth fluocarbonate ores by subjecting the ore to pyrohydrolytic attack in which heated ore is contacted with steam whereby fluorine values in the ore are volatilized and removed therefrom and substantially all of the rare earth values in the ore are converted to acid soluble rare earth oxides which may subsequently be leached from the treated ore. Pyrohydrolytic attack of the ore is generally carried out at temperatures of between 700° C. and 1300° C. Lower temperatures may be used if the ore is digested with a concentrated mineral acid prior to pyrohydrolytic attack.

The present invention relates to the treatment of rare earth fluocarbonate minerals. More particularly, the present invention relates to the treatment of rare earth fluocarbonate ores by pyrohydrolytic procedures.

The treatment of rare earth bearing ores by acid leaching procedures is known. Heretofore, such procedures have not been completely satisfactory when applied to rare earth fluocarbonate ores because it has not been possible to recover more than about 75% by weight of the contained rare earth values, based on the total weight of rare earth values in the ore. The values which were not recoverable by acid leaching techniques were found to be present as acid-insoluble rare earth-fluorine compounds. Attempts to recover these insoluble values have been generally unsuccessful.

In accordance with the present invention, there is provided a process which results in the recovery of substantially all of the rare earth values from fluocarbonate ores, including at least the major portion of the heretofore unrecoverable rare earth values present as acid-insoluble rare earth-fluorine compounds.

It will be understood that the term "rare earth" as used herein includes: those elements of the lanthanide series, having atomic numbers from 57 through 71 inclusive, and the elements yttrium and scandium which may be present in minor amounts in rare earth fluocarbonate ores.

Broadly, the present invention provides a process for the recovery of rare earth values from rare earth fluocarbonate ores, generally bastnasite ores, by subjecting the ore, in particulate form, to pyrohydrolytic attack. At least the major portion of the rare earth values in the particulate ore are converted, by pyrohydrolysis, to acid-soluble rare earth oxides. If desired, pyrohydrolysis of the ore can be preceded by other ore-opening techniques including, for example, pyrolysis to drive off carbon dioxide and convert the rare earth fluocarbonates to rare earth oxyfluorides; leaching with dilute mineral acids to solubilize the alkaline earth carbonate—principally calcium carbonate—portion of the ore; digesting with concentrated mineral acid to dissolve the acid-soluble rare earth values in the ore; or other techniques.

2

The term "pyrohydrolysis" used in this specification, the specific examples and the claims appended hereto, unless otherwise defined means: a decomposition reaction caused by gaseous water and heat. In the pyrohydrolysis of rare earth fluocarbonates, the solid reactants comprise a rare earth material containing an acid-insoluble rare earth-fluoride compound and the reaction products comprise hydrogen fluoride and acid-soluble rare earth oxides.

The term "acid-soluble" as used herein, means, unless otherwise stated, that the identified material is soluble in some concentration of either hydrochloric or nitric acid at a temperature between the boiling and freezing points of the acid mixture under normal atmospheric pressure. Conversely, the term "acid-insoluble" used herein means, unless otherwise stated, that the identified material is substantially insoluble in any concentration of either nitric or hydrochloric acid at any temperature between the boiling and freezing point of the acid mixture under normal atmospheric pressure:

20 The fluocarbonate ore can be subjected to pyrohydrolytic attack as the only recovery procedure to recover substantially all of the rare earth values in the ore as acid-soluble rare earth oxides. If this procedure is followed, the exiting gases from the pyrohydrolytic reaction will

25 contain both carbon dioxide and hydrogen fluoride. Since the carbon dioxide is very volatile and has a very low critical temperature (31.1° C.), it is generally impractical to condense this gas. However, if the carbon dioxide is not condensed, it will carry entrained hydrogen fluoride with it. In order to simplify the recovery of hydrogen fluoride, the pyrohydrolysis preferably is carried out on rare earth fluocarbonate ore after it has been treated to remove at least a major portion of the included carbon dioxide and carbonate.

30 The rare earth oxides recovered from the pyrohydrolysis of rare earth fluocarbonate ores can be utilized as desired. For example, the rare earth oxides may be dissolved in an acid solution to separate the rare earth values from insoluble gangue and to provide the corresponding rare earth salt. The rare earth bearing solution may be separated from the gangue by filtration or other convenient means. Rare earth salt can be separated from the solution by conventional procedures, for example, by evaporation. This rare earth salt may be reduced to the rare earth metal. Rare earth metal may be alloyed with iron as a nodularizing agent. Alternatively, the rare earth salts may be converted to pure rare earth oxides which enjoy wide utility as glass polishing compositions. Individual rare earths may be separated from one another, for

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585

those having the following approximate weight percentage compositions:

|                                 | Percent |
|---------------------------------|---------|
| Fluorine                        | 0.1-9   |
| Rare earths                     | 3-80    |
| Alkaline earth metal carbonates | 1-75    |
| Silica                          | 0.1-25  |
| Barium sulfate                  | 4-50    |
| Iron oxide                      | 1-5     |
| Aluminum oxide                  | 1-5     |

Rare earth fluocarbonate ores of this composition may be found in association with a wide variety of other minerals and valueless gangue materials, some of which may be carried with the fluocarbonate ores into the present process. Such extraneous materials are not generally detrimental to the pyrohydrolysis reaction because the present process can be applied effectively to generally all rare earth fluocarbonate-containing ores.

The rare earth fluocarbonate ores can be subjected to conventional ore-dressing procedures prior to the described pyrohydrolytic attack. Such conventional ore-dressing procedures include, for example, the separation of valueless gangue and other extraneous materials by such techniques as classification, flotation, sedimentation and the like.

The particle size of the rare earth fluocarbonate ore is not critical; however, it is generally possible to increase the rate of reaction by decreasing the particle size, since the surface area, and thus the amount of material exposed to the reaction, increase as the particle size decreases. If the particle size is too large, it is difficult to carry the reaction to completion in a reasonable length of time.

The ore, prior to being subjected to pyrohydrolysis, is preferably treated to reduce its particle size. The particle size of the ore is generally such that it will pass a No. 3 U.S. Standard screen and it may be as small as 1 micron or less. Preferably the particle size of the ore is such that it passes a 100 mesh (U.S. Standard) screen. The conventional ore dressing and sizing operations can be accomplished on commercially available apparatus.

Pyrohydrolytic attack of the rare earth fluocarbonate ore can be accomplished either continuously or batch-wise in commercially available equipment such as, for example, rotary kilns, furnaces, fluidized bed apparatus, and the like.

The pyrohydrolysis reaction preferably is carried out while the ore is maintained at a temperature between 700° C. and 1300° C., preferably between about 900 C. and 1200 C. At about 700° C. the reaction proceeds rather slowly and may not go to completion, while at around 1300° C., care must be taken to avoid producing a solid sintered mass. The optimum temperature for the convenient pyrohydrolysis of any given ore sample is dependent upon such variable as, for example, the composition of the ore, the particle size of the ore, the treatment of the ore prior to pyrohydrolysis and the like. When the ore has been digested with concentrated acid, the pyrohydrolysis reaction proceeds at a lower temperature generally from about 400° C. to 1300° C.

The temperature of pyrohydrolysis should be such that it is sufficient to drive the reaction to substantial completion and render the major proportion of the rare earth values acid soluble in a reasonable period of time. As described more completely hereafter, certain indicators may be relied upon to determine when the reaction is nearly complete. Quantitative analysis of the rare earth values in the solid reactant and reaction product of the pyrohydrolysis reaction will reveal how much of the rare earth value in the solid reactant has been rendered soluble in either nitric or hydrochloric acid by the reaction.

When the major proportion of the rare earth values contained in the ore which were acid-insoluble prior to pyrohydrolysis have been rendered acid-soluble, the reaction is considered to be substantially complete. Preferably,

the pyrohydrolysis reaction is carried to the point at which at least 85% or more of the acid-insoluble rare earth values have been rendered acid-soluble.

Generally, there is a correlation between the total quantity of hydrogen fluoride evolved during the pyrohydrolysis reaction and the completion of the reaction. In general, the reaction is considered to be substantially complete when 85% or more of the fluorine present in the material fed to the pyrohydrolysis reaction has been removed from the reaction mixture as hydrogen fluoride.

Water can be supplied to the pyrohydrolytic reaction at any temperature desired, even as particles of ice; however, it is generally desirable to avoid using low temperature water since it may tend to cool the heated bed of particulate ore below the reaction temperature. Preferably, water is introduced to the pyrohydrolysis reaction in the form of super-heated steam of such a temperature that the cooling effect, if any, of the steam on the mass of heated particulate ore is slight.

If desired, heat can be supplied to the mass of particulate ore through the use of steam which is heated to a temperature above that of the particulate ore. This procedure is often advantageous when the reaction is carried out in a fluidized bed.

Water is generally supplied to the pyrohydrolysis reaction in an amount greatly in excess of that required to react completely with the rare earth and fluorine values in the ore. An excess of water is preferred in order to maintain the maximum rate of reaction.

The time required to complete the pyrohydrolytic reaction, using ore of a given particle size, is largely dependent upon temperature and is determined conveniently by certain observations. Thus, substantial completion of reaction may be determined, for example, by analysis of the solid pyrohydrolysis reaction product and determination of the substantial absence of acid-insoluble rare earth values; or by determination of a substantial decrease in the rate of hydrogen fluoride evolution; or by noting that 85% or more of the fluorine in the solid feed material to the pyrohydrolysis reaction has been removed from the reaction as hydrogen fluoride, silicon tetrafluoride and other volatile fluorine compounds.

At least a part of the carbon dioxide in rare earth fluorocarbonate ores can be removed by pyrolysis prior to pyrohydrolytic treatment. This pyrolysis reaction can be carried out in the substantial absence of water at a temperature above about 500° C. and preferably above about 600° C. or it can be accomplished immediately prior to or concurrently with the pyrohydrolytic reaction in the presence of water. If it is desired to remove any carbon dioxide which may be present in the ore as calcium carbonate, the ore should be heated to a temperature above about 900° C. The fluocarbonate ore is subject to pyrolysis until such time as the evolution of carbon dioxide substantially ceases. The maximum pyrolysis temperature is generally the fusion point of the ore, which is generally above about 1300° C.

If it is not convenient or desirable to remove, by pyrolysis, that portion of the carbon dioxide in the ore which is present as alkaline earth metal carbonate, it can be removed by treating the ore with dilute hydrochloric or nitric acid. Generally, this reaction can be accomplished by admixing the ore with acid until the pH of the mixture declines and remains relatively constant between about 1 and 2. It has been observed that under these conditions, substantially all of the carbonate in the alkaline earth metal carbonate is removed as carbon dioxide and very little, if any, of the rare earth values are solubilized. The completion of this reaction is evidenced by the substantial cessation of gaseous carbon dioxide evolution. This reaction is generally carried out at a temperature between about 20° C. and 50° C.

The pyrohydrolysis reaction may be applied to the insoluble residue from a concentrated acid leach. A concentrated acid leaching step will remove at least a part

of the acid-soluble rare earth values which are present in the ore. A concentrated acid leach step can be accomplished using either nitric or hydrochloric acid at elevated temperatures above about 50° C. and up to the boiling point of the mixture. Generally, the more concentrated the acid, the greater will be the amount of rare earth values solubilized in this step. However, since any rare earth values remaining in the ore after this concentrated leach will be recovered in the pyrohydrolysis reaction, it is unnecessary to impose severe enough reaction conditions to solubilize the maximum amount of acid-soluble rare earth in this step. Conveniently, the acid used in this step can range in concentration from 3 normal to 9 normal or even greater.

Typical analytical procedures for the determination of rare earths may be found in "Treatise on Analytical Chemistry," Kolthoff and Ewing, Part II, volume 8.

General methods for determination of fluorine in bastnasite are given in "Treatise on Analytical Chemistry," Part II, volume 7.

In the specification, claims and following specific examples, all parts and percentages are by weight unless otherwise indicated. The following examples are set forth to further illustrate and not to limit the invention.

#### EXAMPLE I

This example illustrates the optional treatment of rare earth ore with dilute mineral acid to dissolve a portion of the alkaline earth metal carbonate content of the ore before subjecting it to pyrohydrolytic attack.

A bastnasite ore concentrate 90% of which passes a 200 mesh sieve (U.S. Standard) is found to have the following composition:

| Ore components:                          | Weight percent |
|------------------------------------------|----------------|
| * $\text{Ln}_2\text{O}_3 + \text{ThO}_2$ | 57.2           |
| $\text{ThO}_2$                           | 0.03           |
| $\text{CeO}_2$                           | 28.6           |
| $\text{CaO}$                             | 11.3           |
| $\text{MgO}$                             | <0.1           |
| $\text{SiO}_2$                           | 1.2            |
| $\text{SO}_3$                            | 1.2            |
| F                                        | 3.6            |
| $\text{BaO}$                             | 3.9            |
| ** $\text{R}_2\text{O}_3$                | 1.0            |
| Loss on ignition                         | 21.4           |

\*"Ln" is a generic symbol used to represent all of the rare earth elements generally. A mixture of rare earth oxides is present here.

\*\* $\text{R}_2\text{O}_3$ " is a generic symbol used to indicate those compounds which, during systematic analysis, are precipitated from solution by the addition of ammonium hydroxide, and includes iron oxide, aluminum oxide and titanium oxide. Phosphorus pentoxide is co-precipitated with iron oxide and is included here.

A sample of this bastnasite ore composition is admixed with hydrochloric acid solution at ambient temperature. A sufficient quantity of hydrochloric acid solution is used to bring the pH of the mixture down to a constant value of about 1. The undissolved residue is washed twice by decantation, filtered and dried. This dried leached bastnasite ore concentrate contains 72.9 weight percent rare earth oxides, 4.5 weight percent fluorine and has a loss on ignition of 19.6 weight percent. The composition of the mineral bastnasite can be represented by the formula  $\text{LnFCO}_3$ . Using  $\text{CaCO}_3$  to represent the alkaline earth carbonates in general, the principal reactions taking place during this dilute hydrochloric acid leach can be represented as follows:



#### EXAMPLE II

This example is illustrative of the pyrohydrolytic treatment of bastnasite ore which has been leached with acid to remove the alkaline earth carbonates, as in Example I.

The experimental apparatus used consists of a nickel

tube 33 inches long having a 1 inch inside diameter. The first 14 inches of this tube, through which the steam is to be introduced, is enclosed in a preheater which maintains this end of the tube at about 450-480° C. The next 18-inch section of this tube is the main heating furnace in which the temperature is controlled by a resistance heating element capable of maintaining the inside of the nickel tube at any predetermined elevated temperature up to about 1200° C. Steam is introduced into the preheater section where it is heated to a temperature of about 400-480° C. before it passes over a weighed charge of ore in the main heater section. After passing over the ore sample, the steam and gases are passed through a water-cooled condenser and collected for analysis.

The principal reactions taking place during pyrohydrolysis of this leached ore are, first, the pyrolytic reaction:



and, second, the pyrohydrolysis reaction:



In order to analyze the results of this pyrohydrolytic treatment, the solid product remaining in the main heating furnace is treated with an excess of 6 normal hydrochloric acid. This mixture of solid pyrohydrolytic product and hydrochloric acid solution is heated and agitated for about 30 minutes. After this treatment, the insoluble residue is filtered from the solution, dried, ignited to approximately 900° C. and weighed.

The results of carrying out the procedure of this example under slightly different conditions for several different runs are set forth below.

#### Run A

|                                                                            |                                                                                                                           |
|----------------------------------------------------------------------------|---------------------------------------------------------------------------------------------------------------------------|
| Starting material                                                          | 100 g. leached bastnasite.                                                                                                |
| Product of pyrohydrolytic treatment                                        | 76.55 g., a 23.5% loss of weight based on the starting material.                                                          |
| Temperature of main heating furnace                                        | 1200° C.                                                                                                                  |
| Time of pyrohydrolytic treatment                                           | 3 hrs.                                                                                                                    |
| Steam volume                                                               | 3.7-3.8 ml./min. steam condensate.                                                                                        |
| Insoluble residue after leaching the solid pyrohydrolytic reaction product | 1.7 g.; this residue is equal to 2.2% by weight of the pyrohydrolytic product or 1.7% by weight of the starting material. |

105 weight percent of the calculated available fluorine is collected in the steam condensate and 99.5 weight percent of the calculated available rare earth values, calculated as  $\text{Ln}_2\text{O}_3$ , are dissolved in the hydrochloric acid solution.

#### Run B

|                                     |                                                                |
|-------------------------------------|----------------------------------------------------------------|
| Starting material                   | 150 g. of leached bastnasite.                                  |
| Product of pyrohydrolytic treatment | 115.6 g., a 22% loss of weight based on the starting material. |
| Temperature of main heating furnace | 1000° C.                                                       |
| Time of pyrohydrolytic treatment    | 4 hrs.                                                         |
| Steam volume                        | 3.8-4 ml./min. steam condensate.                               |

Insoluble residue after  
leaching the solid pyro-  
hydrolytic reaction  
product ----- 12.35 g.; this residue is  
equal to 10.9% by weight  
of the produce or 8.3%  
by weight of the start-  
ing material.

70 weight percent of the calculated available fluorine is  
collected in the steam condensate and 93.2 weight percent  
of the calculated available rare earth values, calculated  
as  $\text{Ln}_2\text{O}_3$ , are recovered in the hydrochloric acid solution.

*Run C*

Starting material ----- 180.6 g. of leached bast-  
nasite.  
Product of pyrohydrolytic  
treatment ----- 138.2 g., a 23.4% loss of  
weight based on the  
starting material.

Temperature of main heat-  
ing furnace ----- 1100° C.  
Time of pyrohydrolytic  
treatment ----- 5 hrs.  
Steam volume ----- 3.8 ml./min. steam  
condensate.

Insoluble residue after  
leaching the solid pyro-  
hydrolytic reaction  
product ----- 7.44 g., this residue is  
equal to 5.3% by weight  
of the product or 4.3% by  
weight of the starting  
material.

85 weight percent of the calculated available fluorine is  
collected in the steam condensate and 96.8 weight percent  
of the calculated available rare earth values, calculated  
as  $\text{Ln}_2\text{O}_3$ , are recovered in the hydrochloric acid solution.

*Run D*

Starting material ----- 69.8 g. of leached bast-  
nasite.  
Product of pyrohydrolytic  
treatment ----- 54.7 g., a 21.5% loss of  
weight based on the  
starting material.

Temperature of main heat-  
ing furnace ----- 900° C.  
Time of pyrohydrolytic  
treatment ----- 6 hrs.

72 weight percent of the calculated available fluorine is  
collected in the steam condensate and 91.4 weight percent  
of the calculated available rare earth values, calculated  
as  $\text{Ln}_2\text{O}_3$ , are recovered in the hydrochloric acid solution.

*Run E*

Starting material ----- 69.5 g. of leached bast-  
nasite.  
Product of pyrohydrolytic  
treatment ----- 56.1 g., a 19% loss of  
weight based on the  
starting material.

Temperature of main heat-  
ing furnace ----- 800° C.  
Time of pyrohydrolytic  
treatment ----- 4 hrs.

61 weight percent of the calculated available fluorine as  
collected in the steam condensate and 84 weight percent of  
the calculated available rare earth values, calculated as  
 $\text{Ln}_2\text{O}_3$ , are recovered in the hydrochloric acid solution.

**EXAMPLE III**

Prior to pyrohydrolysis the ore used in this example  
is digested with concentrated mineral acid. The digested  
bastnasite is pyrohydrolyzed to recover the rare earth

values in this material which cannot be solubilized with  
mineral acids.

5 A 100 gram sample of leached bastnasite ore concen-  
trate prepared by the method of Example I, above, is  
subjected to attack by 375 ml. of boiling 6 normal hydro-  
chloric acid under reflux for 4 hours. At the end of this  
4 hour period, the insoluble residue is separated from the  
solution and dried. The residue weighs 24.2 grams. Anal-  
ysis shows it to contain 66% rare earths as oxide and  
19.2% fluorine.

10 The residue is subjected to the pyrohydrolytic treat-  
ment, using the same procedure described in Example II,  
above, at a temperature of 1000° C. and a treatment time  
of 3 hours. The product of this pyrohydrolytic attack  
15 weighs 21.0 grams indicating a loss in weight of 13.2%.

This pyrohydrolytic product is digested with an excess  
of boiling 6 N hydrochloric acid. The washed and dried  
15 insoluble product from this leaching step is found to  
weigh 5.2 grams which is 5.2% by weight of the starting  
material.

20 Analysis of the solution obtained from the digestion  
disclose that 14.7 grams or 92% of the rare earth values  
(calculated as rare earth oxide) present in the insoluble  
25 residue prior to pyrohydrolysis are recovered in the leach  
liquid. Rare earth values remaining in the residue  
amounted to 1.28 grams.

Determination of fluorine in the steam condensate  
shows it to contain a total of 4.1 grams which is 90% of  
30 the total contained in the leached bastnasite ore concen-  
trate starting material.

**EXAMPLE IV**

This example is illustrative of the pyrohydrolytic attack  
of bastnasite ore which has not been subjected to a pre-  
35 liminary leach with mineral acid and which has the com-  
position shown in Example I, above.

Twenty grams of unleached bastnasite is heated in a  
tube furnace to 980° C. and 64 ml. of water (as steam)  
are then passed through the tube at a constant rate in a  
40 period of 3½ hours. The product weighs 15.56 grams.  
This product is digested with 100 ml. of 6 normal hydro-  
chloric acid and the insoluble residue from this digestion  
is dried. The dry insoluble residue weighs 1.0 gram.

**EXAMPLE V**

45 This example is illustrative of the optional separate  
pyrolysis treatment to decompose the bastnasite mineral  
and remove carbon dioxide prior to pyrohydrolysis.

50 Fifty grams of leached bastnasite, prepared in Ex-  
ample I, above, are placed in a Vycor tube which is  
connected to a flowmeter. The tube is heated slowly in  
a tube furnace. Slow evolution of gas is noted when the  
temperature of the ore, as shown by a thermocouple  
placed within the furnace, reaches 580° C. Gas evolution  
55 is rapid as the temperature is slowly raised from 600°  
to 640° C., over a period of one hour. The temperature  
is slowly increased for an additional hour and at a tem-  
perature of 690° C. the evolution of gas ceases.

In subsequent pyrolysis reactions, carried out in the  
60 manner described in this example, it is observed that the  
rate of carbon dioxide evolution can be increased by  
increasing the pyrolysis temperature. This temperature  
can be increased up to the sintering point of the ore.

In the subsequent pyrohydrolysis of this pyrolyzed  
65 material, the reaction is initiated at a temperature of  
about 700° C. and proceeds at a commercially practical  
rate at 900° C.

**EXAMPLE VI**

This example is illustrative of the pyrohydrolytic attack  
70 on rare earth fluorocarbonate material which has been sub-  
jected to concentrated acid digestion.

Thirty grams of insoluble residue obtained by the con-  
centrated acid digestion procedure of Example III, above,  
is subjected to the action of water vapor at a tempera-  
ture of 750° C. for a period of five hours. Water is intro-

duced continuously at a rate of 18 grams per hour. The first fractions of condensate collected contain 25 to 33 percent hydrogen fluoride by weight. After 75 minutes, the concentration of fluorine has dropped to 5.2 percent; after 175 minutes, to 2.4 percent; after 240 minutes, to 0.7 percent and after 320 minutes, the fluorine concentration is down to 0.3 percent. At this point, the treatment is terminated.

The product of pyrohydrolysis is digested with 6 N hydrochloric acid. The solution is separated from the small insoluble residue and analyzed. Eighty-seven percent of the rare earth values originally present in the sample prior to pyrohydrolysis is found to be present in the solution as rare earth chloride.

This reaction is repeated to determine the optimum temperature range for carrying out the pyrohydrolysis of rare earth fluocarbonate material which has subjected to a concentrated acid digestion. It is found that pyrohydrolysis begins at 400° C., is fairly rapid at 500° C. and proceeds at a commercially practical rate at 600° C. and higher.

As will be understood by those skilled in the art, what has been described is the preferred embodiment of the invention; however, many modifications, changes and substitutions can be made therein without departing from the scope and the spirit of the following claims.

What is claimed is:

1. A process of treating rare earth fluocarbonate ore which comprises pyrohydrolytically attacking said ore by contacting said ore with steam while the ore is at a temperature of between about 700° and 1300° C. for a period of time sufficient to volatilize a major portion of the fluorine values from said ore and leave a solid product in which a major portion of the rare earth values in said ore have been converted to rare earth oxides which are soluble in inorganic mineral acid.

2. The process as defined in claim 1 in which said ore is contacted with steam which is at a temperature sufficient to heat said ore to a temperature of between about 700° C. and 1300° C.

3. The process as defined in claim 1 in which the ore is heated to a temperature of between about 700° and 1300° C. and is then contacted with steam.

4. The process as defined in claim 1 in which said solid product is admixed with an acid selected from the group consisting of hydrochloric acid and nitric acid to dissolve said rare earth oxides in said acid and produce a liquid mixture containing dissolved rare earth values.

5. The process as defined in claim 1 in which said ore is subjected to pyrolysis prior to said pyrohydrolytic attack by heating said ore to a temperature above about 500° C. in the substantial absence of water to remove at least a portion of the carbon dioxide from said ore.

6. The process as defined in claim 1 in which said ore is admixed with a dilute inorganic mineral acid prior to said pyrohydrolytic attack to remove at least a portion of the carbonate values contained in said ore.

7. The process as defined in claim 6 in which said acid is selected from the group consisting of dilute hydrochloric and dilute nitric acid and said acid is admixed with the ore in an amount sufficient to reduce the pH of said mixture to a value between 1 and 2 to remove substantially all of the carbonate values from the ore prior to said pyrohydrolytic attack.

8. A process for treating rare earth fluocarbonate ore which comprises admixing said ore with a concentrated inorganic acid to form a mixture of solubilized rare earth values and an insoluble residue containing acid insoluble rare earth values, separating said acid insoluble residue from said solubilized rare earth values and subjecting said insoluble residue to pyrohydrolytic attack by contacting said residue with steam at a temperature of between about 400° and 1300° C. for a period of time sufficient to volatilize a major portion of the fluorine values from said residue and leave a solid product in which a major portion of the rare earth values have been converted to rare earth oxides which are soluble in inorganic mineral acid.

9. The process as defined in claim 8 in which said residue is contacted with steam which is at a temperature sufficient to heat said residue to a temperature of between about 400° and 1300° C.

10. The process as defined in claim 8 in which said residue is heated to a temperature of between about 400° and 1300° C. and is then contacted with steam.

#### References Cited

##### UNITED STATES PATENTS

|           |        |       |         |
|-----------|--------|-------|---------|
| 1,129,029 | 2/1915 | Vogt  | 23—16 X |
| 2,735,747 | 2/1956 | Kasey | 23—16   |

##### FOREIGN PATENTS

|         |        |            |
|---------|--------|------------|
| 222,950 | 7/1959 | Australia. |
|---------|--------|------------|

OSCAR R. VERTIZ, Primary Examiner.

H. T. CARTER, Assistant Examiner.